

## UNITED STATES PATENT OFFICE.

WILLIAM R. PATE AND JOSEPH A. GITZEN, OF MILWAUKEE, WISCONSIN, ASSIGNEES  
TO LINDSAY-MCMILLAN CO., OF MILWAUKEE, WISCONSIN, A CORPORATION OF  
WISCONSIN.

## LIQUID CORE BINDER.

No Drawing.

Application filed April 11, 1927. Serial No. 182,998.

This invention relates to a liquid core binder and the process of making the same.

The sand core which is employed in molds for casting metal is composed of sand and a binder.

Among the binders which are employed are powdered rosin and linseed oil.

The rosin produces what is called a rosin or soft core and the linseed oil produces what is called an oil or hard core.

The core is molded from the sand and binder mixed together and then it is heated or baked.

The powdered rosin becomes unified and distributed in the sand while the core is being baked, and then it solidifies after the heat is removed.

The linseed oil dries and solidifies while the core is being baked.

20 The rosin or soft core will yield and allow the casting to shrink and contract and further it is readily removable from the casting as the rosin is softened and then disintegrated by the heat from the molten metal.

25 Powdered rosin, though constituting a binder for core sand which will become plastic when heated to the temperatures involved in core baking and in the casting of metal, has certain decided disadvantages. For ex-

30 ample, rosin is very sticky and hard to maintain in a pulverized form. Consequently, particularly if the room is hot, the pulverized rosin will form into lumps which when mixed with sand by the core maker pro-

35 duces a non-homogeneous mixture, resulting in pockets when the core is baked or when the core is subjected to the action of the molten metal in a mold. When these pockets appear on the exterior of the core, the result

40 is a rough casting. Another disadvantage of the use of powdered rosin as a binder in a core is that the core does not present the strength or toughness required in many operations.

45 The present invention has as its object to

provide a liquid core binder which will be solidified by the heat in baking the core and which will be softened and disintegrated by the heat of the molten metal.

Another object is to provide a liquid core 50 binder which may be readily and economically manufactured.

Another object is to provide a liquid core binder which will readily intermingle with the sand and which will not cause the core to 55 adhere to the mold in which it is formed.

Another object is to provide a core binder which is convenient in use, which may be readily and uniformly mixed with the core sand, which will hold together the particles 60 of the core sand with sufficient tenacity to permit the cores to be handled, and which will permit the necessary disintegration of the core after the casting operation is completed.

65 Another object is to provide a liquid core binder which will become plastic under the temperatures encountered in the casting of metal, whereby shrinkage or other stresses set up during the cooling operation of the 70 casting will not result in the production of destructive stresses to produce cracks in the casting. Expressed in other language, an object of the present invention is to provide a core binder which will produce a core 75 which is plastic under the temperatures encountered in metal casting operations, whereby the core will give, or yield, as shrinkage occurs in the cooling of the cast metal.

Another object is to provide an improved 80 core having the advantages of plasticity and toughness above referred to.

According to this invention as it has been employed in practice, the liquid core binder comprises rosin or other suitable soluble 85 binding matter, petroleum oil or distillate or other volatile solvent, and linseed oil or other suitable strengthening or drying matter, combined in such proportions that the binding matter remains in solution in the 90

solvent under normal temperature and the rosin maintains its fundamental characteristics and constitutes the basic binder.

The liquid core binder provided by this invention has many advantageous characteristics, among which are the rosin is in solution and will readily and uniformly intermingle with the sand, it will be solidified by the heat in baking the core to bind the sand together and hold the core in shape, and it will become plastic and then disintegrate under the heat from the molten metal.

The invention will be further understood and explained from the binder which is set forth in the following composition:

|                                        |     |        |
|----------------------------------------|-----|--------|
| Rosin                                  | 40% | Weight |
| Light petroleum oil 28 Beaumé gravity  | 10% |        |
| Petroleum distillate 40 Beaumé gravity | 44% |        |
| Raw linseed oil                        | 5%  |        |
| Pine oil                               | 1%  |        |

The rosin constitutes the basic binder and it is in solution in the light petroleum oil and the petroleum distillate which are a volatile solvent therefor.

The linseed oil gives the rosin increased strength and tenacity (that is cohesion or toughness) and lessens the rosin required to bind the sand together.

When 40% rosin and 5% linseed oil are present, the binder will have substantially the same strength as 60% rosin alone.

The linseed oil which is employed is insufficient in amount to impair the rosin or overcome its characteristics.

When even about 10% linseed oil is present the rosin will still be the basic binder and maintain its characteristics over the linseed oil.

The pine oil is a ready rosin solvent and promotes maintaining the rosin in solution. The linseed oil, in addition to having drying characteristics to increase the strength and tenacity of the binder, constitutes a solvent for rosin. Therefore, all of the liquids employed with the rosin act cumulatively to hold the rosin in solution.

The solvent retains the rosin in permanent solution under ordinary temperature.

When the core in which the binder is employed is heated and baked, the solvent is volatilized and eliminated and the rosin and the linseed oil therein are solidified to bind the sand together. The distillate distills out with the water in the core sand at the core baking temperatures.

The provision of the petroleum solvents having different boiling points produces the following advantages: The light petroleum oil (which for example may be paraffin oil) permits the melting of the rosin without decomposition thereof. Later on in the baking of the core, said light petroleum oil pro-

tects the rosin, so that if too high a temperature should be used, or baking should be continued for too long a time, the rosin is protected against decomposition. The lighter distillate has the advantage that the mixture is rendered sufficiently fluid to distribute itself uniformly throughout the core sand.

In order to facilitate making the binder and to lessen the volatilization thereof under normal temperature, the light petroleum oil and the petroleum distillate are employed as the solvent.

The light petroleum oil is less volatile than the petroleum distillate, and the petroleum distillate is more fluid and less adhesive than the light petroleum oil.

According to the ordinary process employed to make the binder, the rosin is dissolved under heat which is sufficient to melt the rosin.

When the solution thus obtained is reduced to substantially normal temperature, the petroleum distillate is introduced to make it more fluid and to lessen its adhesiveness.

The linseed oil may be introduced either while the solution is heated or after it is cooled.

The pine oil is introduced after the solution has been cooled.

According to another process for making the binder, the rosin while it is in a heated liquid state in being obtained from its original source is dissolved in the light petroleum oil and then the other ingredients are incorporated in the way which has been set forth.

The term high volatile solvent is employed to comprehend the light petroleum oil which has a higher boiling temperature than the petroleum distillate and the term low volatile solvent is employed to comprehend the petroleum distillate which has a lower boiling temperature than the light petroleum oil.

An important feature of the present invention is that it provides the advantages of rosin in that the core will become plastic under heat (followed by disintegration of the core) as the temperature of the core is raised to a predetermined value. The present invention has the advantage over rosin that, being a liquid, distribution throughout the core sand is more readily and uniformly accomplished. The present invention has the further advantage over dry rosin that the flying powder does not have to be contended with.

The present invention has decided advantages over oil cores (that is, cores comprising sand and core oil or comprising sand and linseed oil,) in that it provides plasticity, whereas oil cores do not have plasticity. An oil core will not soften under heat,

but will finally disintegrate, (though not uniformly) when heated to a sufficiently high temperature. Before disintegration occurs in an oil core, however, shrinkage stresses in the cast metal applied to the non-yielding oil core will, in many instances, produce breakage of the casting. Oil cores, however, by reason of their cheapness, have a field of usefulness in many types of castings where breakage of the castings is not likely to occur, as for example with gray iron castings, which have a relatively low shrinkage modulus, or in castings so designed that the shrinkage is low. The present invention lies in a field distinct from oil cores and constitutes an improvement over rosin cores. The present invention is particularly applicable to the making of castings in which the core should change its shape under the shrinkage of the casting. Castings are practically always provided with apertures which permit the oozing of the plastic core therethrough. Cores manufactured according to the present invention or employing the liquid core binder according to the present invention will disintegrate after the plasticity stage.

The present invention, in addition to the advantage that it is easier than rosin to han-

30 dle, has the further advantage of cheapness in many instances, for the reason that the fluid comprising the present invention permeates the core sand much more readily than does pulverized rosin and is decidedly more efficient as a binder than is pulverized rosin. Therefore, less of the liquid employing the principles of the present invention is required (by weight) for a unit amount of sand than is required of rosin.

40 Added to this advantage is the advantage that no lumps of rosin will collect on the surface of the core, which lumps will fall out either during the core baking operation or thereafter, leaving a rough surface which

45 promotes chafing when the cores contact with one another in storage. Expressed in other language, cores made with liquid employing the principles of the present invention are smoother than rosin cores, and con-

50 sequently will not wear away and crumble as readily as rosin cores. A further ad-

vantage is the smoother casting resulting from the practice of the present invention. Still another advantage of the present in-

55 vention is the reduction of labor cost from the cost involved in the working of rosin, inasmuch as the manipulation of the core binder employing the principles of the pres-

60 ent invention does not have the unpleasant features of flying powdered rosin.

Of course, the composition which has been set forth herein to illustrate the invention and further the process of making the same may be modified in various ways.

65 The invention claimed is as follows:

1. A liquid core binder comprising rosin about forty percent (40%), a volatile solvent about fifty-five percent (55%) and linseed oil about five percent (5%) by weight.

2. A liquid core binder comprising rosin 70 about forty percent (40%), petroleum oil about ten percent (10%), petroleum distillate about forty-five percent (45%) and linseed oil about five percent (5%) by weight.

3. A liquid core binder comprising rosin 75 about forty percent (40%), light petroleum oil about ten percent (10%), petroleum distillate about forty-four percent (44%), linseed oil about five percent (5%) and pine oil about one percent (1%) by weight.

4. A core binder adapted for use with core sand in the manufacture of baked cores comprising a liquid including rosin in a sufficient amount to constitute the essence of said core binder and insure plasticity under 85 metal casting temperatures, and a solvent non-volatile under normal temperatures, said rosin being in solution in said solvent, said solvent including petroleum derivatives and linseed oil.

5. A core binder adapted for use with core sand in the manufacture of baked cores comprising a liquid including rosin in a sufficient amount to constitute the essence of said core binder and insure plasticity under metal 90 casting temperatures, and a solvent non-volatile under normal temperatures, said rosin being in solution in said solvent, said solvent including petroleum derivatives and an oil having drying characteristics.

6. A core resulting from the application of core baking temperature to a mixture of core sand and a binder, which binder is a liquid under normal temperatures and includes rosin in a sufficient quantity to bind the particles of said core into a mass plastic under metal casting temperatures, said rosin being dissolved in a liquid including petroleum derivatives non-volatile at normal temperatures and linseed oil.

7. A core resulting from the application of core baking temperature to a mixture of core sand and a binder, which binder is a liquid under normal temperatures and includes rosin in a sufficient quantity to bind the particles of said core into a mass plastic under metal casting temperatures, said rosin being dissolved in a liquid including petroleum derivatives non-volatile under normal temperatures and an oil having drying 110 characteristics.

8. A core resulting from the application of heat to a mixture of core sand and a binder, which binder contains sufficient rosin to bind the particles of said core sand into a mass plastic under metal casting temperatures, a solvent for said rosin non-volatile at normal temperatures but volatile at core baking temperatures, and an oil having drying characteristics, said oil being in suffi- 125

cient quantity to render said core tenacious and in insufficient quantity to impair the plasticity of said core.

9. A liquid core binder comprising a resinous substance, a solvent therefor non-volatile under normal temperatures, and linseed oil, the linseed oil being about one-eighth of the resinous substance by weight.

10. A liquid core binder comprising a resinous substance dissolved in a mixture of petroleum solvents having different boiling points and non-volatile under normal tem-

peratures and an oil having drying characteristics, said petroleum solvents and said oil having cumulative solvent actions on said resinous substance, said oil being insufficient in quantity to harden said binder beyond a plastic stage at metal casting temperatures.

In witness whereof we have hereunto subscribed our names.

WILLIAM R. PATE.  
JOSEPH A. GITZEN.